

Patented Mar. 27, 1923.

1,449,613

# UNITED STATES PATENT OFFICE.

HIRAM YOUNG McBRIDE, OF DENVER, COLORADO, ASSIGNOR TO THE UNITED STATES WOOL COMPANY, OF DENVER, COLORADO, A CORPORATION OF ARIZONA.

## WOOL CLEANING.

No Drawing. Application filed April 23, 1920, Serial No. 376,130. Renewed May 29, 1922. Serial No. 564,820.

To all whom it may concern:

Be it known that I, HIRAM YOUNG McBRIDE, a citizen of the United States, residing at Denver, in the city and county of Denver and State of Colorado, have invented certain new and useful Improvements in Wool Cleaning, of which the following is a specification.

This invention relates to wool cleaning; and it comprises a method of cleaning raw or greasy wool wherein such wool is agitated for a time with dead burnt gypsum—that is, gypsum or plaster of Paris which has been roasted at a sufficient temperature and for a sufficient time to lose substantially entirely its power for combining with water; all as more fully hereinafter set forth and as claimed.

In the preparation of wool for use in the industries, it is a necessary preliminary step to free the raw wool of the natural grease, suint, or yolk which it contains; a more or less indefinite material containing various water soluble potassium salts, greases and various other organic matters. The wool must also be freed of various other extraneous materials, dirt, etc. Upon the completeness of the removal of these natural impurities depends much of the success of subsequent operations in fabric making. The foreign matters in the wool are, more or less, like a varnish over the surface and this varnish must be removed. The wool fiber has a more or less rough or "serrated" surface, and it is particularly difficult to remove all traces of the foreign matter occurring in the serrations of the fiber. One type of method used for cleaning raw wool is to agitate it with various dry powders. The dirt, wool grease, etc. are taken up by these powders and may be removed with them. While many such powders may be used and certain have been proposed, they do not by any means act alike and it is difficult to secure one which will produce the desired type of thorough-going purification; to secure a material which will effectually remove all the extraneous matter from the wool fibers and which can itself be entirely removed with facility.

One of the best of these pulverulent materials is gypsum, or plaster of Paris, in its various forms. Gypsum, chemically con-

sidered, is  $\text{CaSO}_4 \cdot 2\text{H}_2\text{O}$ ; that is, it is calcium sulfate with two molecules of water of crystallization. By carefully roasting or baking, or as it is frequently termed "calcining," it is converted into ordinary plaster of Paris with the loss of most of its water of crystallization. In the condition in which it is left by this baking or calcining operation, it is able to take up the lost water and reform the original crystallized material; this being the reason that it "sets" with water.

I have found that gypsum may be materially improved as a wool cleaning material by treating it in another manner than that customarily employed in dehydrating. As is well known in the art of making cementitious materials, if the roasting or baking be at too high a temperature and for too long a period, the gypsum not only loses its water but loses the capacity for taking up water again. The roasted material will not set with water. In this condition, which is one that is carefully avoided by those who produce gypsum materials for the trade, the gypsum is known as "dead burnt;" burning has been carried so far that the material remains "dead" in contact with water.

I have found that dead burnt gypsum in contact with greasy wool removes the dirt much more thoroughly than other varieties of gypsum materials. And I find that not only does it take off the grease, etc. from the surface of the fibers but it also removes the grease from the serrations; producing a wool which spins, felts and weaves with unusual facility and which takes dyes and colors much more readily and sharply than otherwise purified wool. As for the reason for the observed superiority of dead burnt gypsum over ordinary gypsum material, I am not certain and content myself with noting the observed fact without committing myself to any theory as to the reasons therefor. I may note however that, whatever the reasons may be, wool cleaning by pulverulent materials is a matter involving, at least to some extent, adsorption phenomena; and adsorption of greasy matters by surfaces which do not contain, and will not take up water, is better than it ever is with moist or hydrated surfaces. But whatever the reason, the fact is as stated: that gypsum

deprived of the power of combining with water by dead burning removes grease, etc. much more effectually than other gypseous materials, even where such material is baked 5 to a substantially anhydrous condition by a baking for a shorter time and at a lower temperature.

One incidental advantage of using dead burnt gypsum for the present purposes 10 which I have noted is that such gypsum does not tend to clump up, since such moisture as is in the wool does not affect it.

In preparing gypsum for my purposes, any ordinary gypseous material of good 15 quality, such as native gypsum, land plaster, plaster of Paris, etc., may be employed. Calcination of some gypsums at a temperature of 500° C. for two hours gives a material suitable for my purposes. I have found it 20 advantageous, in most instances, to calcine the gypsum at about 760° C. for a period of about forty-eight hours—gypsum so calcined has given satisfactory results. Any ordinary type of calcining apparatus adapted 25 for economical treatment of the material at a high temperature may be used. Calcination should be carried on for a sufficient time and at a sufficient temperature to cause the material to lose its power of setting with 30 water; and should be controlled by tests from time to time. The material is best reduced to a powder of at least 250 mesh prior to use.

The powder may be distributed through 35 the wool by any suitable form of agitating device. With a good quality of dead burnt gypsum, it will be found that after the agitation is complete, the gypsum, together with the matters taken up, may be readily

removed by any suitable dusting device of standard type, leaving no residue of either gypsum or grease on the wool. The wool is clean and is ready for manufacturing, etc. In contacting the wool and the dead burnt gypsum, this is best done if the wool is warmed, say, between 100 and 140° F., as this facilitates the action of the dead burnt gypsum in taking up grease, etc.

In practical embodiments of my invention 50 it is advantageous to pick the wool preliminarily in any of the usual devices, adding a little dead burnt gypsum to it during the picking. The picked wool, together with the gypsum, may then be passed through a warm chamber, say, at 100 to 140° F., by means of 55 an imperforate belt. More dead burnt gypsum may be added during this time. Finally the wool may be delivered to a perforate belt in the same chamber. Most of the gypsum and the matter taken up thereby is dropped through the perforations at the bottom of the chamber whence it may be removed by a conveyor or other suitable device. Finally the wool may be freed of the rest of the gypsum, etc., in any ordinary dusting or beating device.

The subject-matter of this application is principally derived from my application Serial No. 142,471, filed Jan. 15, 1917, of which the present application is a continuation in part. 70

What I claim is:—

The process of cleaning wool which comprises agitating such wool with dead burnt gypsum. 75

In testimony whereof, I affix my signature hereto.

HIRAM YOUNG McBRIDE.